

## UNITED STATES PATENT OFFICE

2,116,399

PROCESS FOR MAKING SHAPED BODIES  
FROM HARD SUBSTANCES

Paul Marth, Dusseldorf, Germany

No Drawing. Application November 24, 1936, Serial No. 112,606. In Germany November 29, 1935

3 Claims. (Cl. 75—137)

Up to the present shaped bodies of hard metal-alloys, called "hard metals", were made of carbides, particularly of tungsten carbides, with the aid of more easily fusible auxiliary metals, especially of the iron group, by sintering the powdered mixture of, for instance, tungsten carbide with a carbon content of 3-7% and an additional auxiliary metal or by first forming porous shaped bodies from the powdered carbides by pressing or sintering and filling up the pores with melted auxiliary metals. The sintering of a powdered mixture of carbides and auxiliary metals by means of the so-called compression, under pressure of, for instance, more than 100 kgs./sq. cm., the sintering temperature remaining below the fusion-point of the auxiliary metals, is also known. When treating tungsten carbide by the above-named processes use is made of the finely powdered high-carbon carbide, composed mainly of WC, obtained by carburizing tungsten powder, reduced tungstic acid or ammonium-paramungstate without melting them. The products thus gained have no very great degree of hardness or of resistance to wear. Harder products were obtained by melting tungsten carbides in carbon crucibles or carbon tubes in an electric furnace or between the carbons of the electric arc, the resulting products, however, being extremely brittle and, moreover, very difficult to shape.

The well-known process of sintering together powdered fusion-products obtained in the manner shown above without the use of auxiliary metals also resulted in the production of shaped bodies of insufficient resistance and tenacity.

These disadvantages and difficulties are avoided and an extraordinarily hard and wear-resisting body of sufficient tenacity is produced by heating in refractory moulds, such as carbon moulds, the splintered hard substance gained by melting carbides, nitrides, silicides and borides of metals or metalloids in the presence of atomic hydrogen together with less difficultly fusible metals or metal alloys to temperatures above the fusion-temperature of the binding or bedding metals.

In case of the production of various modifications of the metal or metalloid carbides the use of the low-carbon modifications is advisable. The shaped bodies can be assembled by fusion under compression or they can be compressed prior to this assembly.

Tungsten, molybdenum, titanium, vanadium, zirconium, cerium, silicon, boron, aluminium, beryllium, chromium have proved particularly suitable for the formation of the hard substance,

while the metals of the iron group are used as binding or bedding metals, either by themselves or in the form of their alloys or alloyed, for instance, with vanadium, chromium, tungsten, manganese or molybdenum. By this process the production of shaped bodies is rendered possible without the use of complicated furnaces or equipments. It is sufficient to heat the mould under a gas-blast flame, such as an oxy-acetylene or an oxy-hydrogen flame.

Example.—70% of a splintered low-carbon tungsten-carbide with a carbon content of about 3.7%, which has been melted in the presence of atomic hydrogen, and 30% of bedding material in the form of a crushed tungsten-chromium-cobalt alloy are heated together under pressure in an octagonal refractory mould by means of an oxy-acetylene flame to a temperature beyond the fusion-point of the bedding metal. Shaped bodies made in this way can be used as cutting inserts for core drills and deep-well boring tools.

I claim:

1. A process for producing shaped bodies of an extremely hard substance with a high degree of resistance to wear and of tenacity made from carbides, nitrides, silicides, borides, boron and easily fusible auxiliary metals, which process consists in heating a splintered hard substance obtained by melting material selected from the group consisting of carbides, nitrides, silicides and borides of metals or metalloids in the presence of atomic hydrogen together with binding and bedding material in the form of less difficultly fusible metallic substances in a refractory mould, such as a carbon mould, to temperatures above the fusion-point of the binding or bedding metal.

2. A process for producing shaped bodies consisting of a hard substance which process consists in heating a substance selected from the group which consists of carbides, nitrides, silicides, and borides of elements chosen from the group consisting of tungsten, molybdenum, titanium, vanadium, zirconium, cerium, silicon, boron, aluminium, beryllium, chromium or other similar metals or metalloids forming hard substances which have been melted in the presence of atomic hydrogen together with a metal chosen from the iron group to a temperature above the fusing point of the metal selected from the iron group.

3. A process for producing shaped bodies of a hard substance which process consists in heating a substance selected from the group which consists of a carbide, nitride, silicide or boride

of an element chosen from the group consisting of tungsten, molybdenum, titanium, vanadium, zirconium, cerium, silicon, boron, aluminium, beryllium, and chromium which have been melted in the presence of atomic hydrogen together with a binding agent chosen from the group which

consists of iron alloyed with vanadium, chromium, tungsten, manganese or molybdenum, said heating being at a temperature above the melting point of the melting agent.

PAUL MARTH.